

# United States Patent

Anderson

[15] 3,668,128

[45] June 6, 1972

[54] **ELECTRICAL INSULATING OIL, AND  
TO ELECTRICAL APPARATUS  
INCORPORATING THEM**

[72] Inventor: John Kenneth Anderson, Bexley, England

[73] Assignee: British Insulated Callender's Cables  
Limited, London, England

[22] Filed: Jan. 2, 1970

[21] Appl. No.: 461

[30] **Foreign Application Priority Data**

Jan. 9, 1969 Great Britain ..... 1,298/69

[52] U.S. Cl. ..... 252/63, 117/154, 117/201,  
174/25, 203/14

[51] Int. Cl. ..... H01b 3/00

[58] **Field of Search** ..... 252/63; 208/14; 174/25;  
117/154, 201

[56] **References Cited**

UNITED STATES PATENTS

3,163,705 12/1964 Feick ..... 252/63

|           |        |                |          |
|-----------|--------|----------------|----------|
| 3,573,209 | 3/1971 | de Dryver..... | 252/63   |
| 3,318,799 | 5/1967 | Acker.....     | 252/63 X |
| 2,719,182 | 9/1955 | Ross.....      | 252/63 X |
| 2,870,385 | 1/1959 | Rice.....      | 252/63 X |
| 2,921,011 | 1/1960 | Ordelt.....    | 252/63 X |
| 2,993,156 | 7/1961 | Robinson.....  | 252/63 X |

*Primary Examiner*—Robert F. Burnett

*Assistant Examiner*—M. E. McCamish

*Attorney*—Buell, Blenko and Ziesenhein

[57] **ABSTRACT**

An insulating oil which has good resistance to oxidation and which is also non-gassing and of low viscosity comprises from 1–50 percent (by weight) of a residually unsaturated alkene polymer, and correspondingly from 99–50 percent of a low viscosity hydrocarbon oil. The polymer is derived predominantly from an alkene or alkenes having from three to five carbon atoms and has an average molecular weight in the range 100–900, preferably in the range 250–500. A mixture of such alkene polymers may be used. The hydrocarbon oil is preferably a mineral oil, and has a viscosity of 30 centistokes or less at 20° C.

17 Claims, No Drawings

## ELECTRICAL INSULATING OIL, AND TO ELECTRICAL APPARATUS INCORPORATING THEM

The present invention relates to electric insulating oils and more especially, but not exclusively, to oils based on selected and refined mineral oils. The invention is especially concerned with oils for use in the impregnation of the dielectric of power cables (chiefly paper-insulated power cables) and of other electrical apparatus, such as capacitors and transformers.

In order to obtain a low power factor and a high degree of resistance to oxidation, it is desirable to use a mineral oil having a low aromatic content. At the present time mineral oil having an aromatic content of less than about 7 percent is not readily available, and it is preferable that the aromatic content should be as close as possible to this figure, and preferably below it if and when such oil becomes available. However, it is found that mineral oils of low aromatic content have a tendency to evolve gas, predominately hydrogen, under the influence of an electric field, contributing to the formation of gas-filled voids in which discharges occur, leading to degradation and ultimately to complete breakdown of the insulation. Similar difficulties arise with some types of synthetic hydrocarbon oil.

Such "gassing" is reduced and preferably avoided by adding to the oil a constituent which will react with and so absorb nascent hydrogen, and oils containing such a constituent are known, and will hereinafter be referred to, as "non-gassing." The added constituent will for convenience be referred to as "the additive."

Hitherto, when an oil of low viscosity (e.g., below 40 centistokes at 20° C.) was required, aromatic additives, conventionally naphthalenic extracts of petroleum, have been used, with the result that the power factor of the oil was raised, and its oxidation resistance decreased.

In accordance with the present invention, an insulating oil which has good resistance to oxidation and which is also non-gassing and of low viscosity comprises from 1-50 percent (by weight) of a residually unsaturated alkene polymer derived predominately from an alkene or alkenes having from three to five carbon atoms (or a mixture of such alkene polymers) the or each polymer having an average molecular weight in the range 100-900, and correspondingly from 99-50 percent of a low viscosity hydrocarbon oil which has a viscosity of 20 centistokes or less at 20° C., and would gas if used alone.

The hydrocarbon oil is preferably a refined mineral oil which is preferably predominately naphthenic in character or of mixed naphthenic/paraffinic composition, and preferably of low aromatic content. Naturally, a mineral oil having a low power factor and high oxidation resistance is preferred.

In addition to propene, butylenes and/or amylenes, the alkene polymer may include a small number of units derived from ethylene and/or from higher alkenes. Polymers derived predominately from butenes are preferred.

The average molecular weight of the alkene polymer is preferably below 700 and more especially in the range 250-500. An average molecular weight of about 350 is suitable.

The preferred amount of the additive depends, subject to satisfactory non-gassing properties, upon its molecular weight and upon the viscosity desired. When the molecular weight of additive is in the preferred range of 250-500, addition of from 5-15 percent is suitable for oils for use in oil-filled cables having internal oil channels, and from 10-40 percent for oils for use either in accessories of such cables or in pipe-type cables.

The invention includes electrical apparatus comprising a body of porous and/or laminated insulating material impregnated with the oils described; it further includes oil-filled paper insulated electric cables in which the paper is impregnated with the oils described.

The principal advantages of the insulating oils in accordance with the invention may be summarized as follows:

- the amount of additive required for any desired degree of gas absorption is less than when conventional additives of the aromatic type are used;
- the viscosity of the oil can be controlled at a low value;

- the additive has no appreciable deleterious effect and may on the contrary have a beneficial effect on the oxidative stability or electrical properties of the oil;
- the additive is formed as a by-product in the manufacture of alkylene polymers of high molecular weight, and is therefore relatively inexpensive;
- the low temperature hydraulic behavior of the oil is good, and in particular its pour point is not unduly raised; and,
- under conditions of electric stress, the oil is less sensitive than conventional oils to the presence of traces of moisture.

In the following tables, oils A and D are examples of selected refined naphthenic mineral base oils, sold by the Burmah Oil Trading Co., Dussek Division under the designations T3252 and T 3251 respectively, oils B, B1 and E examples of oils in accordance with the invention for oil-filled cables of the type having internal oil channels and oils C and F examples of accessory oils in accordance with the invention. The polybutene additive in oils B, C, E and F is a commercial polybutene sold under the Trade Name POLYVIS OO and having an average molecular weight of 350 and a viscosity at 20° C. of 120 centistokes. The polybutene additive in Oil B1 is another commercial polybutene having an average molecular weight of 300.

TABLE I

| Oil                                    | A        | B            | B1           | C                     |
|----------------------------------------|----------|--------------|--------------|-----------------------|
| Mineral Oil Content                    | 100%     | 90%          | 87%          | 70%                   |
| Polybutene additive content            | Nil      | Oil A 10%    | Oil A 13%    | Oil A 30%             |
| Viscosity (CS) at 20°C.                | 5.5      | 6.0          | 6.0          | 11                    |
| 60°C.                                  | 2.0      | 2.3          | 2.3          | 3.6                   |
| Specific Gravity at 20°C.              | 0.86     | 0.86         | 0.86         | 0.85                  |
| Flash Point (closed cup) °C. (Typical) | 110      | 110          | 110          | 110                   |
| Pour Point °C.                         | -85      | -75          | -75          | -64                   |
| Gassing character in range 0°-130°C.   | evolving | non-evolving | non-evolving | Strongly non-evolving |

TABLE II

| Oil                                    | D        | E            | F                     |
|----------------------------------------|----------|--------------|-----------------------|
| Mineral oil content                    | 100%     | 90%<br>Oil D | 70%<br>Oil D          |
| Polybutene additive content            | Nil      | 10%          | 30%                   |
| Viscosity (cS) at 20°C.                | 14       | 17           | 27                    |
| 60°C.                                  | 4.5      | 5.2          | 6.2                   |
| Specific gravity at 20°C.              | 0.88     | 0.87         | 0.86                  |
| Flash point (closed cup) °C. (Typical) | 130      | 130          | 28                    |
| Pour Point °C.                         | -65      | -62          | -57                   |
| Gassing character in range 0°-130°C.   | evolving | non-evolving | Strongly non-evolving |

What I claim as my invention is:

- An insulating oil which has good resistance to oxidation and which is also non-gassing and of low viscosity comprising a. from 1-50 percent by weight of at least one residually unsaturated alkene polymer having an average molecular weight in the range 100-900, and derived predominately from at least one alkene having from three to five carbon atoms and

- b. correspondingly from 99-50 percent of a low viscosity hydrocarbon oil which has a viscosity of 30 centistokes or less at 20° C. and would gas if used alone.
- 2. An insulating oil as claimed in claim 1 in which the molecular weight of said alkene polymer is in the range 100-700.
- 3. An insulating oil as claimed in claim 2 in which the molecular weight of said alkene polymer is in the range 250-500.
- 4. Electrical apparatus comprising a body of insulating material impregnated with the insulating oil claimed in claim 1.
- 5. An oil-filled paper insulated electric cable in which the paper is impregnated with the insulating oil claimed in claim 1.
- 6. An insulating oil which has good resistance to oxidation and which is also non-gassing and of low viscosity comprising
  - a. from 1-50 percent by weight of at least one residually unsaturated alkene polymer having an average molecular weight in the range 100-900, and derived predominately from at least one alkene having from three to five carbon atoms and
  - b. correspondingly from 99-50 percent of a low viscosity refined mineral oil having a viscosity of 30 centistokes or less at 20° C.
- 7. An insulating oil as claimed in claim 6 in which said alkene is butene.
- 8. An insulating oil as claimed in claim 6 in which the molecular weight of said alkene polymer is in the range 100-700.

15

20

25

25

- 9. An insulating oil as claimed in claim 8 in which the molecular weight of said alkene polymer is in the range 250-500.
- 10. An insulating oil as claimed in claim 9 suitable for use in accessories of oil-filled cables having internal oil channels and for use in pipe-type cables and comprising from 10-40 percent of said alkene polymer.
- 11. An insulating oil as claimed in claim 9 suitable for use in oil-filled cables having internal oil channels comprising from 5-15 percent by weight of said alkene polymer, and correspondingly from 95-85 percent of said low viscosity refined mineral oil.
- 12. An insulating oil as claimed in claim 11 in which said alkene polymer is a polybutene.
- 13. An oil-filled paper-insulated electric cable in which the paper is impregnated with the insulating oil claimed in claim 11.
- 14. An insulating oil as claimed in claim 6 in which the refined mineral oil is predominately naphthenic in character.
- 15. An insulating oil as claimed in claim 6 in which the refined mineral oil is of mixed naphthenic/paraffinic composition.
- 16. Electrical apparatus comprising a body of insulating material impregnated with the insulating oil as claimed in claim 6.
- 17. An oil-filled paper insulated electric cable in which the paper is impregnated with the insulating oil claimed in claim 6.

\* \* \* \* \*

30

35

40

45

50

55

60

65

70

75